

# UNITED STATES PATENT OFFICE.

FRIEDRICH EDUARD BÖTTIGER, OF OFFENBACH-ON-THE-MAIN, GERMANY, ASSIGNEE  
TO THE CORPORATION OF CHEMISCHE FABRIK GRIESHEIM-ELEKTRON, OF FRANK-  
FORT-ON-THE-MAIN, GERMANY.

## TREATMENT OF MERCERIZED COTTON GOODS.

1,002,026.

Specification of Letters Patent. Patented Aug. 29, 1911.

No Drawing.

Application filed July 24, 1909. Serial No. 509,377.

To all whom it may concern:

Be it known that I, FRIEDRICH EDUARD BÖTTIGER, doctor of philosophy, chemist, a subject of the German Emperor, and resident of Offenbach-on-the-Main, in the Grand Duchy of Hessen, Germany, with the post-office address Ludwigstrasse No. 9, have invented new and useful Improvements Relating to the Treatment of Mercerized Cotton Goods, of which the following is a specification.

A crackling feel is given to mercerized cotton goods by working them in a soap bath and souring afterward. If in this process goods are used, which have been dyed with sulfurized dyestuffs, the color-acid of these dyestuffs is liberated by the action of the acid used in the souring process. The sulfur of the dyestuff then becomes oxidized to sulfuric acid gradually or at once according to the conditions. This acid tenderers or even disintegrates the cotton fiber on prolonged storage, hot pressing, shrinking and finishing of hosiery. To avoid this tendering of the fiber an addition of 5 to 10 grams of sodium acetate per liter of acid bath (10 grams of acetic acid per liter) has been proposed in the United States specification No. 693653, in English specification No. 2972 of 1901 and in French specification No. 308238. The prescribed quantity of sodium acetate prevents the deterioration of the fiber only partly as will be shown by the following statement. A yarn (20/4 Maco) dyed with sulfur black lost 75.82 per cent. of its original tensile strength by the process of giving it a crackling feel by means of acetic acid (10 grams per liter) and steaming afterward (one hour at 1½ atmospheres), 30.42 per cent. by addition of 5 grams of sodium acetate per liter acid bath and 8.59 per cent. by addition of 10 grams sodium acetate. To preserve completely the tensile strength of the cotton fiber an addition of a larger proportion of sodium acetate must be made to the acid bath. On applying such large proportions of sodium acetate in the process however a crackling feel cannot be produced. On addition of 10 grams of sodium acetate per liter the crackling feel will be very feeble, on addition of 15 grams it cannot be perceived any more. Therefore this process is not fit to produce the scroop of silk on

mercerized cotton goods, dyed with sulfurized dyestuffs, without reducing the tensile strength of the fiber.

According to the present invention a crackling feel can be imparted to cotton by means of hydroxy-carboxylic acids of the aliphatic series, to wit: lactic or tartaric acid, by the addition of such proportions of the salts of the said acids or by partly neutralizing the said acids to such a degree that the cotton fiber may not be tendered. How much of the acid has to be neutralized or how much lactate or tartrate has to be added to the acid bath depends on the intensity of the dyeing, on the sulfurized dyestuff used in the dyeing process, and on the proportion of acid added to the bath. If in the process of imparting a crackling feel to cotton goods, dyed with 10 per cent. of thioxin black, 5 grams of lactic acid for instance are to be used, about 15 grams of sodium lactate or 17 grams of lactic acid and 7 grams of anhydrous sodium carbonate or 22.4 grams of caustic soda lye of 30° Baumé specific gravity, must be added per liter.

The best results in carrying out the new process are obtained if one part of the acid used in the after treatment of the mercerized cotton, dyed with sulfurized dyestuffs, 3 to 5 parts of its salts are added.

As the acids mentioned in the said specifications are not suitable for producing a crackling feel on mercerized cotton, dyed with sulfurized dyestuffs, without weakening the tensile strength of the fiber, the particular action of the acids and their salts employed according in this invention for imparting the scroop of silk to cotton goods without reducing the tensile strength of the fiber could not be foreseen.

The method of applying this invention will be illustrated by the following examples.

Example I. 50 pounds of mercerized cotton yarn are dyed in the usual manner with a black sulfurized dyestuff for instance thioxin RTo, rinsed and worked in a soap bath containing 5 to 10 grams of soap per liter. The yarn is hydro-extracted without being rinsed and treated in a bath containing 17 grams of lactic acid and 7 grams of anhydrous sodium carbonate or 22.4 grams of caustic soda lye 30° Baumé specific grav-

ity. The yarn is worked in this partly neutralized bath for 15 to 20 minutes hydro-extracted without being rinsed and dried. The yarn thus treated acquires a good crackling feel and the original tensile strength of the fiber is not altered by steaming under pressure or on prolonged storage. Instead of lactic acid and sodium carbonate or caustic soda lye 5 grams of lactic acid and 15 10 grams of sodium lactate may be used to obtain the same result.

Example II.—The process is carried out according to Example I but instead of lactic acid 21.3 grams of tartaric acid or 5 grams 15 tartaric acid and 25 grams of sodium tartrate and 11.5 grams of anhydrous sodium carbonate or 36.7 grams caustic soda lye 30° Baumé specific gravity may be used per liter of dye bath.

I claim:

1. The process of giving the scroop of silk to mercerized cotton goods, dyed with sulfurized dyestuffs, consisting in souring

the goods, after a passage through a soap bath with a hydroxy-carboxylic acid of the 25 aliphatic series in presence of a salt of said acid, wherein to one part of the used acid 3 to 5 parts of a salt of this acid are added, substantially as described.

2. The process of giving the scroop of 30 silk to mercerized cotton goods dyed with sulfurized dyestuffs, consisting in souring the goods, after a passage through a soap bath with lactic acid in presence of a salt of this acid, wherein to one part of lactic acid, 35 used in the process, 3 parts of a lactate are added, substantially as described.

In testimony, that I claim the foregoing as my invention, I have signed my name in presence of two witnesses, this thirteenth 40 day of July, 1909.

FRIEDRICH EDUARD BÖTTIGER.

Witnesses:

JEAN GRUND,  
ROBERT BÜHL.